

May 13, 1924.

N. H. HOLLAND

1,493,631

DIAPHRAGM AND METHOD OF MAKING THE SAME

Filed Nov. 28, 1921

Fig. 1.



Fig. 2.



Fig. 3.



Fig. 4.



Fig. 5.



Fig. 6.



Inventor:  
Newman H. Holland,  
by Jas. L. Palmer  
ATTY.

## UNITED STATES PATENT OFFICE.

NEWMAN H. HOLLAND, OF WEST ORANGE, NEW JERSEY, ASSIGNOR TO WESTERN ELECTRIC COMPANY, INCORPORATED, OF NEW YORK, N. Y., A CORPORATION OF NEW YORK.

## DIAPHRAGM AND METHOD OF MAKING THE SAME.

Application filed November 28, 1921. Serial No. 518,254.

To all whom it may concern:

Be it known that I, NEWMAN H. HOLLAND, a subject of the King of Great Britain, residing at West Orange, in the county of Essex, State of New Jersey, have invented certain new and useful Improvements in Diaphragms and Methods of Making the Same, of which the following is a full, clear, concise, and exact description.

10 This invention relates to diaphragms and particularly to those intended to be used for acoustical purposes.

An object of the invention is to provide an acoustical diaphragm of light mass and of 15 uniform structure.

Another object is to provide a process of making light diaphragms which is comparatively inexpensive and one by which the characteristics of the product may be accurately controlled.

Other objects appear hereinafter.

The invention, in general, comprises an electro-deposited diaphragm, preferably formed by electro-depositing a metal on a 25 disc consisting of a metal ring and a core of dissimilar material, which is removed after plating, leaving the diaphragm attached to the ring.

30 The advantages of extremely light diaphragms are recognized in the art of sound reproduction but the difficulty of obtaining uniform product and of handling them without damaging has made their use very expensive. Heretofore, the most successful

35 light diaphragms have been those made by rolling metal very thin. In working the metal, however, internal stresses are introduced which cause warping. In view of this and the difficulties which are experienced in

40 mounting such diaphragms, it has been necessary to provide special means for clamping and tensioning them to obtain the desired characteristics. Necessarily the thickness of such diaphragms is controlled by the

45 mechanical strength required to permit its being tensioned sufficiently to remove any warping and regional strains, whereas diaphragms in accordance with the present invention need be only of sufficient thickness

50 to support their own weight or that of any parts that may be mounted thereon.

In the drawings, Fig. 1 represents a complete diaphragm, part of which is in section.

Figs. 2, 3 and 4 represent different stages in the process of making the diaphragm.

Figs. 5 and 6 represent modified forms in cross section.

In the process of making the diaphragm in accordance with the invention, a ring 7 has its opening closed by a filler 10 which may be either conductive in itself or have its surface coated with some conducting material. One surface of the filler and the ring is prepared in the usual manner for electro-plating, the face 15 of ring 7 and the face 16 of filler 10 being flush. The assembly, shown in Fig. 3, is then placed in a suitable plating bath and a continuous plate covering the surface 15 and 16 is deposited by any well known electro-plating process and the thickness of the plate regulated in the usual manner. After the plating is completed, the filler 10 is removed leaving the diaphragm 8 attached to ring 7, as in Fig. 1.

Fig. 5 shows a modification in which an electrode 11 is attached to the diaphragm in the plating process, the electrode 11 being embedded in the filler so as to be flush with surfaces 15 and 16. In the case of the diaphragm intended for use on a receiver, the member 11 may be of magnetic material or the diaphragm itself may be of electro-deposited iron. As stated above, the diaphragm may be made of any desired thickness, and it also may be made of a number of superimposed electro-deposits of different materials as shown exaggerated in Fig. 6 by plates 12, 13 and 14.

It is evident therefore, that diaphragms having practically any desired characteristics may be obtained simply by controlling the plating process. The accuracy and the facility with which the plating process may be controlled makes it possible to produce diaphragms of more nearly identical characteristics than can be produced by any other known method. This invention therefore, eliminates the difficulties which have heretofore been experienced in making extremely thin diaphragms.

While a flat diaphragm is shown in the drawing for the purpose of illustrating the invention, it is obvious that diaphragms of any desired shape such as conical or corrugated, may be made by forming the surface of the filler to correspond to the shape de-

sired. It has also been found convenient to permit the plating to extend over the marginal surface of the ring instead of only on the front surface as shown. However, this is a detail which may be controlled in a well known manner in the plating process.

What is claimed is:

1. A diaphragm comprising an annular member and a sheet of thin material electrolytically attached thereto closing the opening therein.

2. An acoustical diaphragm comprising an annular member, a second member within said annular member, and a sheet of thin metal electrolytically attached to both members.

3. An acoustical diaphragm comprising an annular member, a second member, one face of each member lying in the same plane and in concentric relation, and an electro-plate deposit on each member continuous therebetween.

4. The process of making an acoustical diaphragm which consists in the plating of an annular member and a conducting filler in

said member, and then removing said filler leaving the plate spanning the opening in said ring.

5. The process of making an acoustical diaphragm which consists in filling the opening in a ring with a conducting material, preparing one face of the filler and ring so as to present a smooth plane surface, depositing an electro-plate on said surface and then removing said filler leaving the deposited metal across the opening in said ring.

6. The process of making an acoustical diaphragm which consists in filling an annular member with conducting material, embedding in said filler a plate concentric with said member, preparing one face of the ring, filler and plate so as to present a smooth plane surface, depositing a metal uniformly on said surface, and then removing said filler leaving said plate across the opening between said plate and member.

In witness whereof, I hereunto subscribe my name this 23rd day of November A. D., 1921.

NEWMAN H. HOLLAND.